

# UNITED STATES PATENT OFFICE.

RADCLYFFE FURNESS, OF JENKINTOWN, AND RICHARD H. PATCH, OF PHILADELPHIA, PENNSYLVANIA, ASSIGNORS TO THE MIDVALE STEEL COMPANY, OF PHILADELPHIA, PENNSYLVANIA, A CORPORATION OF PENNSYLVANIA.

## TOOL-STEEL ALLOY.

1,206,834.

Specification of Letters Patent.

Patented Dec. 5, 1916.

No Drawing.

Application filed January 19, 1916. Serial No. 72,901.

To all whom it may concern:

Be it known that we, RADCLYFFE FURNESS and RICHARD H. PATCH, citizens of the United States, residing at, respectively, 5 Jenkintown, county of Montgomery, State of Pennsylvania, and Philadelphia, county of Philadelphia, State of Pennsylvania, have invented a new and useful Improvement 10 in Tool-Steel Alloys, of which the following is a full, clear, and exact description.

The object of our invention is to produce a new and improved high speed tool steel having a substantially higher efficiency than 15 known tool steels to which it is most analogous.

A high speed tool steel containing about 5% of chromium, about 18% of tungsten, about 1% of vanadium, and about 4% of 20 cobalt, is known. A high speed tool steel of the following composition is also known: chromium from 2.5 to 4%, tungsten from 16.5 to 20%, vanadium from 1 to 2%, and cobalt from 3 to 7%. Other tool steels containing the same ingredients with slightly 25 different proportions are also known. These tool steels are very efficient, but they are so expensive that other less expensive tool steels of less efficiency are very frequently 30 preferred. We have discovered, however, that a tool steel employing the above ingredients may be rendered both less expensive and at the same time more efficient by a partial substitution of cobalt for tungsten 35 within certain limits. Thus, we have discovered that if the tungsten be displaced by cobalt until the cobalt reaches 10%, the efficiency of the tool steel will be actually doubled; while if the cobalt is increased to 40 15%, the efficiency will be nearly tripled, that is, will be about 275% of the efficiency of the tool steels hereinbefore mentioned. Above 15% the increased efficiency imparted by the cobalt increases at a pronouncedly 45 reduced ratio, so that the increased efficiency of steel containing cobalt beyond 18 or 20% does not compensate for the increased cost.

While we have spoken of displacing the tungsten by cobalt, we do not mean to be 50 understood as asserting that the tungsten must be reduced to the exact extent that the cobalt is increased, it being impracticable to reduce the tungsten to below about 9%.

Inasmuch as under present conditions the price of tungsten is nearly six times that 55 of cobalt, it will be understood that our improved tool steel is much less expensive, even though the cobalt be increased out of proportion to the decrease of tungsten; and that even under normal conditions, during 60 which the price of cobalt somewhat exceeds that of tungsten, the greatly increased efficiency of our improved tool steel makes it actually more economical.

We contemplate employing varying percentages of the several ingredients of our improved composition within the following ranges: chromium 2 to 6%; tungsten 9 to 15%; cobalt 5 to 20%; and vanadium 1 to 2%. The vanadium may be dispensed with, 70 inasmuch as its addition does not change the essential characteristics of the tool steel, although its incorporation in the composition somewhat improves it. The carbon content of the tool steel may vary from 75 .55% to .75%.

A preferred composition is as follows: chromium 4%; tungsten 13.5%; vanadium 1.5%; cobalt 15%; iron 65%; carbon .65%; with traces of other ingredients usually 80 present in steel.

While it has been heretofore suggested that the percentage of cobalt in tool steels of the character of those herein referred to may range as high as 15 per cent.; no information is given, in connection with such statement, with respect to the proportions of chromium and tungsten to be used therewith, and still less has there been any suggestion of the discovery, underlying our 90 present invention, that cobalt may profitably displace tungsten, or of the extent to which such displacement is practicable, or of the fact that by such substitution, within the limits specified herein, the efficiency of the tool steel will not only be increased, but multiplied, and with an actual diminution in cost.

While we have mentioned that the steel above described is adapted especially for 100 high speed tool steel, it is also capable of other uses, as for example any device for working hot metal, such as gripper dies, nut piercers and header dies. For such purposes the steel should contain from 20 to 105 .60 per cent. of carbon.

Having now fully described our invention, what we claim and desire to protect by Letters Patent is—

1. A high speed tool steel containing 5 chromium 2 to 6%, tungsten 9 to 15%, and cobalt 5 to 20%.
2. A high speed tool steel containing from 2 to 6% chromium, less than 15% of tungsten, and not less than 10% of cobalt.

In testimony of which invention, we have 10 hereunto set our hands at Philadelphia, Penna., on this 15th day of January, 1916.

RADCLYFFE FURNESS.  
RICHARD H. PATCH.

Witnesses:

HARRY D. SIEGFRIED,  
Jos. ENTWISLE.